

Feb. 7, 1961

H. M. ZIMMERMAN ET AL

2,971,044

CORROSION INHIBITORS

Original Filed Jan. 3, 1956



*Fig. 1.*

*Fig. 2.*



*Fig. 4.*

*Fig. 3.*

INVENTORS  
HERMAN M. ZIMMERMAN  
ROBERT A. POWERS

BY *John F. Heimann*  
ATTORNEY

2,971,044

## CORROSION INHIBITORS

Herman M. Zimmerman and Robert A. Powers, Lakewood, Ohio, assignors to Union Carbide Corporation, a corporation of New York

Original application Jan. 3, 1956, Ser. No. 557,013, now Patent No. 2,900,434, dated Aug. 18, 1959. Divided 10 and this application June 9, 1959, Ser. No. 819,034.

9 Claims. (Cl. 136—161)

This invention relates to corrosion inhibitors adapted for use in primary cells, particularly dry cells, and to cells containing such inhibitors.

Open circuit corrosion of dry cell anodes when the cells are on shelf or in storage or at rest during intermittent discharge is a problem which has troubled the dry cell industry from its inception. The unwanted consequences of this problem are perforation of the container anode, shortening of shelf life, and reduced service capacity. To cite but one example of its seriousness, in the case of telephone cells, approximately 50 percent as much zinc is removed from the anode by wasteful corrosion as by useful, current-producing, anodic attack.

To prevent or lessen such corrosion, many expedients have been suggested and tried, including the introduction in various ways of mercury, mercury salts and chromic salts in the cell.

Among the disadvantages of using mercury or mercury salts alone as cell corrosion inhibitors are the following:

(1) Zinc possesses metal impurities having low hydrogen overvoltage, which tend to accumulate on the anode surface during operation, with the net result that the overvoltage of the amalgam surface is lowered while the corrosion rate increases.

(2) The effectiveness of amalgamation is limited by the extent to which air can be excluded from the cell.

(3) As corrosion is a surface reaction, only that mercury present at the anode-electrolyte interface is effective in reducing corrosion.

(4) Mercury must be uniformly distributed at the anode surface. Non-uniform amalgamation can arise in many ways in a dry cell, and lead to high corrosion rates.

(5) Because of its embrittling effect on conventional anodic materials, only very small amounts of mercury can be used. This is true regardless of whether mercury or mercuric salts are employed.

Chromate inhibitors often prove unsatisfactory, as these are affected by the presence and nature of cell paste, and often lose their effectiveness during operation.

Previous work using cationic organic compounds as dry cell corrosion inhibitors has shown them to be unsatisfactory in that they tend to form high resistance anode films or react with cell components, although wasteful anode corrosion may be low.

Lately it has been recognized that marked improvements in dry cell behavior with respect to corrosion inhibition can be obtained with inhibitors having several technical characteristics.

(1) Corrosion inhibiting materials should not react detrimentally with either electrolyte or cell mix.

(2) These should be of such form as always to be available at the anode in a proper concentration.

(3) These should inhibit wasteful corrosion without reducing the anode effectiveness.

In line with this realization and with a view to obviating prior art limitations, the principal object of the present

invention is to provide corrosion inhibitors having novel and improved characteristics.

A further object of the invention is to provide a dry cell having substantially improved properties attributable to the incorporation therein of the corrosion inhibitors of the invention.

Seeking to attain these objects, we have discovered that non-ionic surface active compounds made by the addition of ethylenic oxide compounds to hydroxyl-bearing compounds, effectively inhibit wasteful corrosion by raising the hydrogen overvoltage at the anode of the cells in which they are incorporated without adversely affecting normal cell performance.

In the drawings:

15 Fig. 1 is a sectional elevational view of a conventional paste-lined cell containing the compounds of the invention;

Fig. 2 is a sectional elevational view of a film-lined cell having the herein-disclosed additives;

20 Fig. 3 illustrates an external cathode cell to which the corrosion inhibitors of this invention have been added; and

Fig. 4 is a sectional elevational view of a flat-type or "stacked" cell with the compounds of the invention.

25 The addition compounds which successfully perform in the practice of the invention generally possess the formula  $R-O(R')_n-R''$ , where  $R$  stands for alkyl, aryl or aryl alkyl radicals, where  $R''$  may be either hydrogen or a grouping similar to  $R$ ,  $R'$  is an alkoxy radical such as ethoxy or propoxy, and  $n$  may be any number between 1 and 50. These compounds are essentially linear polymers having wetting characteristics. Their inhibiting properties result from high hydrogen overvoltage created on the anode surface.

30 35 Examples of the above compounds with their effect on hydrogen overvoltage are presented in Table I.

Table I

|    | Class of Starting Material     | Actual Starting Material                                                    | Moles Ethylene Oxide Added | Relative Over-voltage |
|----|--------------------------------|-----------------------------------------------------------------------------|----------------------------|-----------------------|
| 40 | Polynuclear, Aromatic Phenols. | p-phenyl phenol.....                                                        | 6 to 27                    | 1.0                   |
|    |                                | 2-naphthol.....                                                             | 12                         | 1.0                   |
|    |                                | 1-naphthol.....                                                             | 11                         | 1.0                   |
|    | Phenyl Substituted Alcohols.   | Triphenyl Methanol.....                                                     | 14                         | 0.5                   |
| 45 | Alkyphenols.....               | Nonylphenol.....                                                            | 4 to 28                    |                       |
|    |                                | Octylphenol.....                                                            | 4 to 40                    | 0.3 to 0.7            |
|    |                                | Isooctylphenol.....                                                         | 10                         |                       |
| 50 | Phenol.....                    | Phenol.....                                                                 | 8                          | 0.5                   |
|    |                                | 2-ethyl hexanol.....                                                        | 13                         | 0.5                   |
|    | Aliphatic Alcohols.....        | (starter on either end of polyoxyethylene chain).<br>2,6,8-trimethyl-4..... | 8                          | 0.2                   |

55 Virtually all non-ionic surfactants of this type can raise the hydrogen overvoltage. Maximum overvoltage effects result, however, from polyoxyethylated polynuclear aromatic phenols and alkyl aryl phenols. As little as 0.05 percent by weight of electrolyte or anode-contacting media of these materials suffice to satisfactorily prevent wasteful cell corrosion.

60 The corrosion inhibitors of this invention may be used alone or mixed.

The corrosion inhibiting compounds of the invention may be incorporated in a cell by mixing with electrolyte 65 or with the depolarizing mix, or in conjunction with the separator paste or film liner. Their effectiveness, however, is not affected by the method of introduction, as long as they are rendered immediately available to the anode surface.

70 To provide an understanding of the invention, and for conciseness, it will be described mainly by illustrations

of the performance of two compounds of the non-ionic type. The first of these, known as parahydroxydiphenyl polyethylene oxide, also is known as paraphenyl phenoxy polyethylene glycol, hereinafter is referred to as "PPPG." This material is made by the addition of thirteen equivalents of ethylene oxide to one equivalent of parahydroxydiphenyl. Its nominal structure is as follows:



The second compound described is known as Neutronyx-600, and is characterized as an alkylphenol polyglycol ether. This material is prepared by reacting approximately nine and one-half moles of ethylene oxide with one mole of nonylphenol.

Other specific materials of the same general type which have been tested and found to be suitable corrosion inhibitors for dry cell use are:

- (1) Polyglycol ether of 1-naphthol (containing 11 equivalents of ethylene oxide).
- (2) Polyglycol ether of 2-naphthol (containing 12 equivalents of ethylene oxide).
- (3) Polyglycol ethers of p-phenyl phenol (containing 6, 13, 15, 18 or 27 equivalents of ethylene oxide).
- (4) Polyglycol ether of triphenylmethanol (containing 14 equivalents of ethylene oxide).
- (5) Polyglycol ethers of nonylphenol (containing approximately 4, 6, 10, 11, 15, 30 or 40 equivalents of ethylene oxide).
- (6) Polyglycol ethers of octylphenol (containing approximately 3, 5, 7 or 9 equivalents of ethylene oxide).
- (7) Polyglycol ether of phenol (containing 8 equivalents of ethylene oxide).
- (8) Polyglycol ether of di(2-ethyl hexanol) (containing 13 equivalents of ethylene oxide).
- (9) Polyglycol ether of 2,6,8-trimethyl-4-nonyl (containing 8 equivalents of ethylene oxide).
- (10) Glycol ether of octylphenol (containing 1 equivalent of ethylene oxide).
- (11) Polyalkyl ether of dodecylphenol (containing 75 weight percent of mixed ethylene and propylene oxides).

Referring again to the general formula above, it is seen that R may stand for the residue of an initially hydroxyl compound.

Fig. 1 represents a conventional dry cell having a container anode, preferably of zinc 10, an insoluble cathode, preferably of carbon 12, an electrolyte-wet depolarizing mix consisting of manganese dioxide 14 and cereal paste 16 intermediate the anode and cathode. The cereal paste, in this case, contains about 0.05 percent by weight of p-phenyl phenoxy polyethylene glycol 18.

Fig. 2 is a conventional film-lined D-size round cell having a consumable container anode 20, preferably of zinc, an insoluble cathode 22, usually of carbon, an electrolyte-wet depolarizing mix 24 and an anode-contacting film 26 intermediate the anode and cathode. In this case the film has been modified by the incorporation therein of about 0.05 percent "PPPG."

To incorporate "PPPG" in D-size round cells, the standard procedure for making anode-contacting films was slightly modified. Two and three-tenth grams of "PPPG" liquid were placed in hot, rapidly agitated, distilled water. To this stirred solution was added 9.52 grams of water-soluble 4000 cps. methyl cellulose. Stirring was continued until all the methyl cellulose was wet. The resulting solution was then cooled in an ice bath with continued stirring to maintain a uniform thickness, and until all the methyl cellulose dissolved. The solution was then poured on to a horizontal 300 square inch glass plate provided with a removable brim of plastic tape, and allowed to dry. The resulting film was about 0.0015 inch thick. A 2 1/4 inch by 4 inch portion of it was placed between the barrier layer and the zinc anode in several D-size cells. Table II below indicates a breakdown of

solution and dried film composition and cell usage of anode films containing mercury and "PPPG" as zinc corrosion inhibitors for use in D-size cells.

Table II

|    | Film Identification                                                                                                                                          | Hg Control                  | "PPPG"                      |
|----|--------------------------------------------------------------------------------------------------------------------------------------------------------------|-----------------------------|-----------------------------|
| 10 | Solution Composition:<br>Water..... grams..... 600<br>4,000 cps. water-soluble methyl cellulose..... 9.52<br>"PPPG"..... none<br>Mercuric chloride..... 0.75 | 600<br>9.52<br>2.30<br>none | 600<br>9.52<br>2.30<br>none |
|    | Total grams soln./300 sq. in. plate.....                                                                                                                     | 610.27                      | 611.82                      |
| 15 | Film Composition/sq. in. Dry Anode Film:<br>4,000 cps. water-soluble methyl cellulose..... milligrams..... 31.75<br>"PPPG".....<br>Mercuric chloride.....    | 31.75<br>2.50               | 31.75<br>7.65               |

## FILM USED PER D-SIZE CELL

|    |                                  |                   |
|----|----------------------------------|-------------------|
| 20 | Total film area per cell.....    | 10.828 sq. in.    |
|    | Total film size per cell.....    | 2 1/4 x 4 1/8 in. |
|    | Total active film area/cell..... | 7.25 sq. in.      |
|    | Total active film size/cell..... | 1 3/4 x 4 in.     |
|    | Total film thickness.....        | 0.0015 in.        |

25 Fig. 3 shows an external cathode cell comprising a non-corrodible tube 30, composed of fibrous material such as wrapping paper, a cathode 32 of electrically conductive carbon composition molded in situ, an anode 34, preferably composed of zinc, centrally located in the cell, and provided with radial veins, and an electrolyte-wet depolarizing mix in the space intervening between the anode 34 and the cathode 32 at 36. The electrolyte in this instance contains about 0.05 percent by weight of "PPPG."

30 The flat type battery of Fig. 4 comprises an outer container 40 containing a plurality of thin dry cells, such as 42, composed of an electrolyte-wet depolarizing mix 43, an anode-contacting film 44, a zinc anode 46 and a carbon cathode 48. The electrolyte has been modified in accordance with the method of the invention, by the addition thereto of 0.05 percent by weight thereof of "PPPG."

35 In the above cell, as in previous ones, the additive of the invention may be varied in accordance with the scope of the invention. Again the quantity of additives may be modified without departing from the scope of the invention.

Table III

| Example No. | Depolarizer                        | Inhibitor           | Zinc Cans Used      | Initial |       |
|-------------|------------------------------------|---------------------|---------------------|---------|-------|
|             |                                    |                     |                     | Volts   | Amps. |
| 55          | Electrolytic Manganese Dioxide, do | Hg..... "PPPG"..... | Soldered, alloy, do | 1.59    | 9.4   |
|             |                                    |                     |                     | 1.52    | 7.7   |
| 60          |                                    |                     | 12 Months           |         |       |
| 65          | Example No.                        | Volts               | Amps.               | Cm.     | Volts |
|             |                                    |                     |                     |         |       |
| 1.....      | 1.48                               | 4.1                 | 44                  | 1.48    | 3.4   |
| 2.....      | 1.44                               | 4.2                 | 55                  | 1.47    | 4.4   |
| 18 Months   |                                    |                     | Cm.                 |         |       |

60 It is apparent that the use of "PPPG" obviates the need for using pure zinc in cell constructions. Accordingly, this material may be substituted for mercury. A poorer grade or thinner gage of zinc may be incorporated in cell constructions to reduce cost and to conserve materials scarce in critical times, if the organic inhibitors are used. At least 10 percent less zinc may be used if the instant inhibitors are employed.

Results comparable with those discussed for film lined cells were obtained also with D-size paste-filled cells, wherein eight and one-half milligrams of another effective agent, Neutronyx-600, per ten milliliters of paste have been added.

The disappearance of external indications of corrosion (perforation of zinc cans) and the smoother surface of the active inside surface indicated that the inhibitor was extremely effective for reducing general zinc corrosion as well as eliminating areas of excessive corrosion up to ages of 24 months.

The experiments with Neutronyx-600 offer evidence that the benefits derived from non-ionics such as "PPPG" and Neutronyx does not reside mainly in their function as wetting agents.

The exact mechanism whereby the desired effects obtain is not known. The interaction between "PPPG" and zinc affords a hypothesis. Taking electron diffraction patterns of an abraded zinc surface before and after contact with a 1 percent solution of "PPPG" in benzene, it was observed that a definite amount of "PPPG" is firmly adsorbed by the zinc surface. The amount thus retained appears less than a full mono-layer, and is oriented with respect to the metal surface. This and other data indicate that "PPPG" is both chemically and physically adsorbed by zinc, and the observed increase in hydrogen overvoltage of zinc may be attributed to such an adsorbed layer. However, regardless of any theory of operation, our experiments highlighted in the present disclosure have proven that the service life of cells is very materially increased for any service in which shelf life is an important factor.

The inhibitors of this invention find successful employment in various types of primary cell structures. Naturally, for best performance, optimum variations may be made from the foregoing disclosure without departing from the spirit and scope of the instant invention.

This application is a division of our co-pending application Serial No. 557,013, filed January 3, 1956, now Patent No. 2,900,434.

What is claimed is:

1. In combination in a primary dry cell having a consumable anode, an insoluble cathode, an electrolyte-wet depolarizing mix and at least one organic corrosion inhibitor in contact with said anode, said organic inhibitor being defined by the formula



wherein R is at least one radical selected from the group which consists of alkyl, aryl and aryl alkyl radicals, R' is an alkoxy radical, n is any number between 1 and 50, and R'' is at least one radical selected from the group which consists of hydrogen, alkyl, aryl and alkyl aryl radicals.

2. In combination in a primary cell having a consumable anode, an insoluble cathode, an electrolyte-wet depolarizing mix, separator means intermediate said anode and cathode, said separator means containing an organic corrosion inhibitor in contact with said con-

sumable anode, said organic inhibitor being defined by the formula



5 wherein R is a radical selected from the group consisting of alkyl, aryl and aryl alkyl, R' is an alkoxy radical and n is a number between 1 and 50, and R'' is at least one radical selected from the group which consists of hydrogen, alkyl, aryl and alkyl aryl radicals.

10 3. In combination in a primary cell having a zinc anode, a carbon cathode, a depolarizer mix consisting of manganese dioxide and at least one organic corrosion inhibitor in contact with said zinc anode, said organic inhibitor being defined by the formula



wherein R is at least one radical selected from the group consisting of alkyl, aryl, and aryl alkyl radicals, R' is an ethoxy radical and n is a number between 1 and 50, and R'' is at least one radical selected from the group which consists of hydrogen, alkyl, aryl and alkyl aryl radicals.

15 4. In combination in a primary dry cell having a zinc anode, an electrolyte-wet manganese dioxide depolarizer mix, a carbon cathode and corrosion inhibiting means consisting of p-phenyl phenoxy polyethylene glycol dispersed in said cell, contacting said zinc anode.

20 5. In combination in a primary dry cell having a zinc anode, carbon cathode, an electrolyte-wet manganese dioxide depolarizer mix, separator means intermediate said anode and cathode, said separator means containing p-phenyl phenoxy polyethylene glycol to inhibit wasteful corrosion of said zinc anode.

25 6. In combination in a primary cell having a zinc anode, an insoluble cathode, an electrolyte-wet depolarizing mix consisting of manganese dioxide, cereal paste intermediate said anode and cathode, said cereal paste containing p-phenyl phenoxy polyethylene glycol to inhibit wasteful corrosion of said zinc anode.

30 7. In combination in a primary cell having a zinc anode, an insoluble cathode, a depolarizing mix consisting of manganese dioxide and an electrolyte containing p-phenyl phenoxy polyethylene glycol to inhibit wasteful corrosion of said zinc anode.

35 8. In combination in a primary cell having a zinc anode, an insoluble cathode, a depolarizing mix consisting of manganese dioxide and an electrolyte containing at least about 0.05 percent by weight of an alkyl-phenyl polyglycol ether.

40 9. In combination in a primary cell having a zinc anode, a cathode, a depolarizing mix consisting of manganese dioxide, and an electrolyte containing at least about 0.05 percent by weight of a polyoxyethylated polynuclear aromatic phenol to inhibit the wasteful corrosion of said zinc anode.

45 55 References Cited in the file of this patent  
UNITED STATES PATENTS  
2,900,434 Zimmerman et al. Aug. 18, 1959